

E. J. HICKSON,  
MANUFACTURE OF STEEL SHEATHED TUBING,  
APPLICATION FILED JUNE 12, 1915.

1,205,742.

Patented Nov. 21, 1916.

FIG. 1.



FIG. 2.



WITNESS:

*J. Robert Bradley.*

INVENTOR.

*E. J. Hickson*  
*J. Robert Bradley*

ATTORNEY

# UNITED STATES PATENT OFFICE.

EDWIN J. HICKSON, OF BUTLER, PENNSYLVANIA.

## MANUFACTURE OF STEEL-SHEATHED TUBING.

1,205,742.

Specification of Letters Patent. Patented Nov. 21, 1916.

Application filed June 12, 1915. Serial No. 33,693.

To all whom it may concern:

Be it known that I, EDWIN J. HICKSON, a citizen of the United States, and resident of Butler, in the county of Butler and State 5 of Pennsylvania, have invented certain new and useful Improvements in the Manufacture of Steel-Sheathed Tubing, of which the following is a specification.

The method of the present invention is 10 directed to the manufacture of sheathed tubing, and has particular reference to applying a sheathing of polished steel or equivalent material to a tubular or other core of relatively inexpensive steel or iron without 15 distorting the sheathing or injuring or marring its surface.

While the product of the present invention is designed primarily for use in metal bed frames, it may be used wherever material 20 of this nature may be utilized to advantage, and obviously the invention is not restricted to applying the sheathing to a tubular core, nor to a core of any particular cross-sectional shape.

Brass sheathed tubing is extensively used, 25 particularly in the manufacture of metal beds, the sheathing and tubular core being ordinarily drawn through steel dies which shape the sheathing closely to the core, and 30 by the same operation the longitudinal edges of the sheathing are seamed and interlocked, this without injuring the finished surface of the sheathing. In attempting to similarly 35 apply thin and polished steel sheathing, the considerable friction between the sheathing and the steel dies caused by the high pressure 40 incident to the die operation has resulted in so dragging, distorting and marring the sheathing as to render the product unfit for use. Also, the heat resulting from 45 such friction sets up an amalgamating tendency between the like metals of the sheathing and dies that is an important damaging factor. So far as I am informed, polished 50 steel sheathed tubing has not heretofore been successfully manufactured, at least by a process wherein the sheathing and core are united when in a cold state and with the surface of the sheathing given its ultimate finish prior to applying it to the core.

The method of the present invention entirely overcomes the difficulties noted as by means thereof I am enabled to produce polished sheathed tubing without flaw or blemish 55 and at the same manipulation cost as

that incident to the manufacture of brass sheathed tubing.

The essential feature of the invention is the provision of dies formed of a metal that will neither distort nor amalgamate with 60 the thin steel sheathing nor mar its polished surface under the pressure necessary to conform and secure the sheathing to the core. I successfully accomplish this result by the use of dies formed of brass, the steel 65 sheathed tubing thus produced being as perfect in every particular as the best quality of brass sheathed tubing. In shape or contour the dies are no different from steel dies used in the brass sheathing process, 70 and the method of manipulating the core and sheathing does not differ from the familiar practices incident to the manufacture of brass sheathed tubing, the core and the thin and highly polished ribbon-like sheath- 75 ing being passed through the dies in the usual manner and the edges of the sheathing are seamed and jointed together by any of the seaming or jointing devices well known in the trade.

While I have successfully practised the new method by the use of brass dies, I do not confine myself thereto as the invention contemplates dies formed of any other metal or alloy which will accomplish the same result in the application of thin and polished 80 steel sheathing to a metal core.

Apparatus for practising the invention may be variously embodied. An adaptation of mechanism, largely diagrammatic, is illustrated in the accompanying drawings, 85 wherein—

Figure 1 is a view in longitudinal section of dies suitable for the purpose, and Fig. 2 is a view illustrating portions of the core 90 and sheathing before and after they have been united.

In the drawings, A designates an initial or forming die, and B and C, respectively, 100 are finishing dies through which the material passes after emerging from die A. The dies may be mounted in any suitable frame or head conventionally illustrated at D, and a portion E at the front of the latter may be utilized as a support for any 105 suitable seaming or jointing device, not shown.

F designates a metal core, here shown of tubular form, and G is a sheathing of thin and highly polished steel which is passed to 110

the dies in ribbon form, as is customary in the manufacture of brass sheathed tubing.

Various devices are well known in the art for seaming and jointing the longitudinal edges of the sheathing after the latter has been conformed to the metal core, and I therefore deem it unnecessary to illustrate any particular form of jointing or seaming mechanism.

10 It will be understood that the disclosures in the accompanying drawings are of a very general character, and that in practice, the invention is not limited to any particular form or arrangement of dies, so long as they 15 are formed of a metal that will accurately apply the sheathing to the core without distorting it or marring its smooth and polished surface.

I claim:

20 1. The method of producing sheathed cores which consists in longitudinally bringing together the core and a ribbon of thin sheet steel and while cold drawing the core and ribbon of steel through finishing means 25 composed of brass or equivalent material that will force the steel ribbon to inclose and tightly conform to the core without distorting or marring the surface of the steel, substantially as described.

30 2. The method of producing sheathed cores which consists in bringing together the core and a ribbon of thin sheet steel having its exterior surface previously 35 polished, and drawing the core and steel ribbon through tube conforming metallic means of higher specific gravity than steel that will not amalgamate with the polished surface of the steel ribbon in the presence of heat and pressure incident to such drawing, substantially as described.

Copies of this patent may be obtained for five cents each, by addressing the "Commissioner of Patents, Washington, D. C."

3. The method of tightly inclosing cores in steel sheathing to produce steel sheathed tubing having a smooth and polished outer surface, which consists in applying a ribbon of thin sheet steel having a smooth and polished exterior surface to the core, and longitudinally drawing the core and steel ribbon through forming and finishing dies, the finishing dies being composed of metal of different density and softness than steel and that will not amalgamate with steel under heat and pressure incident to such drawing, substantially as described.

4. The method of producing sheathed cores which consists in longitudinally bringing together a cold core and a ribbon of cold thin sheet steel having a smooth outer surface, and drawing the core and steel ribbon while held under compression by copper alloy conforming means that will force the steel ribbon to tightly inclose the core without distorting or marring the smooth surface of the steel.

5. The method of permanently and tightly inclosing cores in steel sheathing to produce steel sheathed tubing having a smooth outer surface, which consists in longitudinally applying to the core when cold a ribbon of thin cold sheet steel having a smooth exterior surface, and folding the ribbon around the core and drawing the core and steel ribbon through a finishing die composed of copper alloy, substantially as and for the purposes described.

In testimony whereof I affix my signature in presence of two witnesses.

EDWIN J. HICKSON.

Witnesses:

FRANK R. FROST,  
L. ROWLEN.